

## UNITED STATES PATENT OFFICE

ROBERT WILHELM STREHLENERT, OF NOL, SWEDEN

## FUEL AND METHOD OF MAKING SAME

No Drawing. Application filed June 16, 1927, Serial No. 199,399, and in Sweden May 18, 1926.

The present invention relates to a method the purpose of which is to manufacture fuel in an economical way from two different kinds of waste products obtained in two different branches of industry and each of which is considered as rather onerous. The waste products that are here in question are on the one hand those obtained in saw-mills and other works in which wood is being worked mechanically or chemically, chiefly in the shape of chips, shavings, dust and the like, hereinafter referred to as saw-dust, and on the other hand those which in the form of waste sulphite liquor are obtained in the manufacture of sulphite cellulose. Although many ways have been suggested to utilize these waste products no way has as yet been found to be of any value prior to the present invention.

20 Saw-dust has been burnt in the saw-mills or other works with rather uneconomical result, principally more for the removal or destruction of the same than for utilizing the low heat energy content of it. Attempts 25 have also been made to make fuel briquets of saw-dust, but such attempts have as yet met without success in manufacturing such briquets of sufficient strength.

With regard to the sulphite liquor it is 30 known that it can be decomposed to form a so-called sulphite fuel whereby, however, only about 70%, according to hitherto known methods, are recovered. It is known also to use sulphite liquor as a liquid fuel. Compared with market prices of coal the price 35 of sulphite fuel will be rather high, and the use of the sulphite liquor as a liquid fuel does not give a result economical enough for an extensive use.

It is also known to use the sulphite liquor as a binding material in making briquets of coal-dust or brown coal-dust and in the manufacture of building materials for different 45 purposes. As an example of this may be cited such methods as are described for instance in Swedish Patents Nos. 14364 and 45359.

By the present invention it is possible to 50 prepare a suitable material from said two

waste products by a method by means of which there is obtained a satisfactory fuel as respects economy and whereby all the substance in the liquor that can be solidified is utilized. According to this method the saw-dust is preferably dried to complete dryness. The sulphite liquor which is to be mixed with and fully absorbed by the saw-dust, is in any known manner evaporated to a concentration of 25 to about 60% dry substance, or 55 the sulphite liquor may also be added successively to the saw-dust in which case the water in the liquor is evaporated while mixing the substances. These two substances are mixed in an ordinary mixing apparatus, 60 which takes only a very small amount of power. I have found that when the sulphite liquor is absorbed by the fibrous wood substance the salt in the liquor remains in the wood cells, while the water in which the salt 65 has been dissolved escapes through the cellular tissue of the fibrous wood substance. The quantity of dry substance contained in the finished dry product and derived from the liquor may vary and may be 25 to 60% of the 70 finished mass. A mixture containing about equal parts of the both substances in the finished product gives, however, a very advantageous result. The mixing operation will 75 be best done if the mass then contains about 36% water. If sulphite liquor of higher or lower concentration is used it is better to keep the amount of water in the mixture at about 36%. The mixture is in no respect 80 of a viscous consistency, as the liquor is very well absorbed by the saw-dust, and it may 85 with advantage be dried to a desired degree of dryness in a drying drum.

It is known to use sulphite liquor as a binding material. In order to obtain suitable 90 briquets it is, however, required, as has been found in working out this invention, that in making the same the binding has to be almost momentary. In a case like this such a binding cannot, however, take place under other 95 conditions than those under which the mixture is dried to about nearly the limit of dryness. Even in such a case the liquor does not bind the saw-dust particles sufficiently together if the mass just before the pressing opera- 100

tion has not been steamed whereby the same is softened, and nor is it possible to obtain a briquet of sufficient density to sustain a certain pressure unless a steamed mass is employed.

A mass with said consistency cannot, however, be treated with steam in the same way as in ordinary steaming, that is to say, by blowing steam into the mass as such, as a uniform moistening would thereby not be obtained and the liquor furthermore would disengage from the saw-dust and the entire mass would be of a pasty consistency. For this reason the mass must according to this invention be steamed in the following manner. The mixture of liquor and saw-dust after having been dried so as to contain only a few percent of moisture is during its transport to the briquet press precipitated into a chamber, for instance a drum, a pipe conduit or the like, of suitable depth and into which at the bottom thereof is blown saturated steam. The short time that it takes the mass to pass said chamber on its way to the briquet press is, however, sufficient for a partial condensation of the steam upon the particles of the mixture and also sufficient for the necessary heating of the same. The mass takes up only about 2% of water, but this is sufficient in order to soften the liquor in such a degree that, when the mass arrives to the briquet press, it is in a condition to be compressed and at once may be pressed as a homogenous briquet so that the same does not later expand or crack. The pressing of the briquets is performed in warm matrices.

The quantity of liquor residue contained in the briquets has firstly the purpose of raising the value of the briquet as a fuel, and besides it increases its density and serves also as a binding material between the particles of the saw-dust and furthermore it makes the briquets unaffected by changes in atmospheric conditions, if the briquettes after having left the press are subjected to a drying carbonizing process at about 200° C., the liquor residue is changed into an insoluble composition which in addition to conserved binding power still more increases the calorific power of the briquets.

Briquets manufactured in accordance with the method above described and at a pressure of about 600 kg. per Cm<sup>2</sup>, have a density between 1.4 and 1.5 which is about the weight of coal. Having left the press the briquets may be used at once as a fuel for steam boilers or in other fire places, where high calorific value is required, or may be treated as above described.

If eventually subjected to a carbonizing process, the dry liquor in the briquets assists to reduce the cost of heating as the dry liquor during the decomposition, which takes place during the heating process is exothermic, thus contributing to raise the temperature, or in

other words the heat of reaction is sufficient for the carbonization process when the proportion between dry liquor and saw-dust is as above specified. This carbonization process is thus not to be confounded with before known carbonization processes for briquets and the like, as in a carbonization process where the percentage of liquor constitutes such a great part, as above specified, for carrying out the method in question, the dry liquor is in the first place acting as an introducer and then as a source of heat for the carbonization process.

Instead of manufacturing briquets of the mass of liquor and saw-dust as prepared for this purpose said mass may also be used for the manufacture of a pulverous fuel.

It is well known that pulverous fuels emanating from a solid product of a more or less valuable calorific content if being injected in the fire place give a considerably higher effect, and this effect will be higher the more the material is finely divided.

Of course the briquets manufactured according to this invention may like other solid fuel be crushed to a pulverous fuel of which product results a technical effect that is proportionate to the degree of fineness of the particles, but such a process is always rather expensive.

The material of which briquets are manufactured as above described may also, if desired, according to this invention be used for the manufacture of a pulverous fuel. The costs for carrying out the method for manufacturing such fuel are less than the costs for manufacturing the briquets. The method of manufacturing the pulverous fuel consists therein that the mass of sulphite liquor and saw-dust without being steamed is subjected to the same process as the briquets, when these are heated to 200° C. when all the liquor product in the mass at the same time is transformed into an insoluble state.

As above indicated, an exothermic reaction takes place during the said heating process acting in such a way upon the wood substance in the mass that this latter will loose its structure and be broken up in an amorphous powder or so changed in its nature, that the mass when subjected to some slight mechanical action will fall asunder in an amorphous powder.

The powder thus obtained is not to be confused with a crushed product which always has to be estimated by the size of the particles. The amorphous powder obtained according to this invention is formed during the course of the chemical reaction which takes place during the decomposition of the liquor product and the action upon the wood substance.

An amorphous mass thus produced and emanating from the constituent parts of the

wood, lignin and cellulose, burns when injected in a fire place, and especially if pre-heated air then is used, like a combustible gas or oil and is of a thermal efficiency which is quite comparable with the efficiency of these last named materials.

It is evident that the fuel in the amorphous state cannot be used anywhere and in all different places but is to be used when convenient. The briquets, which have a high weight of volume and thus are easy to transport, have their special market.

For the manufacture of one ton raw briquets or one ton amorphous powder there is required 580 kg. dry saw-dust and 4200 kg. ordinary waste sulphite liquor containing about 10% dry substance or a corresponding greater or less quantity of liquor depending upon the degree of dry substance contained in the same.

It is evident that instead of saw-dust there may be used finely divided wood obtained in any other way than by sawing.

Briquets in accordance with this invention may be manufactured at a price of about half the present price of coal and the amorphous powder at a price that is still considerably lower.

Having now described my invention what I claim as new and desire to secure by Letters Patent is:

1. The process of preparing a fuel from waste sulphite liquor and sawdust which comprises mixing sawdust with a waste sulphite liquor in such concentration and proportion that the mixture on a dry basis contains about 25 to 60% dry materials derived from the sulphite liquor, partly drying the resulting mixture, heating the partly dried mixture with live steam to raise the temperature of the mixture and to moisten the mixture, forming the moistened mixture into briquettes under pressure and thereafter drying and heating the briquettes at a temperature not substantially in excess of 200° C.

2. In the process of preparing a fuel from waste sulphite liquor and sawdust, the steps which comprise heating to about 200° C. a dried mixture prepared by mixing sawdust with a sulphite liquor in such concentration and amount that the mixture on a dry basis contains about 25 to 60% of dry materials derived from the sulphite liquor.

3. A fuel consisting of a baked mixture of sawdust and dried sulfite liquor the latter forming 25% to 60% of the mixture.

4. A briquet consisting of a baked mixture of sawdust and dried waste sulfite liquor, the latter ingredient forming 25% to 60% of the mixture.

5. A fuel consisting of a baked mixture of sawdust and dried sulfite liquor, the latter forming 25% to 60% of the mixture, said mixture being in an amorphous state.

6. In the process of preparing a fuel from waste sulfite liquor and sawdust, the steps

which comprise heating to about 200° C. a dried mixture prepared by mixing sawdust with a sulfite liquor in such concentration and amount that the mixture on a dry basis contains about 25 to 60% of dry materials derived from the sulfite liquor in order to obtain an amorphous material.

In witness whereof I have hereunto set my hand.

ROBERT W. STREHLENERT.

70

75

80

85

90

95

100

105

110

115

120

125

130